# EUROPEAN PATENT APPLICATION

(11) **EP 0 445 291 A1**
(43) Date of publication of application: **11.09.1991**
(21) Application number: 89911395.5
(22) Date of filing: 13.10.1989
(51) Int. Cl.: B41M 5/30, B41M 5/40

(54) **HEAT-SENSITIVE RECORDING PAPER**

(30) Priority: 28.09.1989 JP 253094/89
(71) Applicant: HONSHU PAPER CO., LTD., Chuo-ku Tokyo (JP)
(72) Inventor: SASAKI, Keiji, Tokyo-to 133 (JP); MORONUKI, Katsumi, Koganei-shi, Tokyo-to 184 (JP)
(74) Representative: VOSSIUS & PARTNER
(86) International application number: JP8901055
(87) International publication number: WO9104869

(57) **Abstract**

In heat-sensitive recording paper having a heat-sensitive coloring layer containing a colorless or light color leuco compound and a developer causing coloration of the leuco compound upon heating on a support, this invention relates to heat-sensitive recording paper wherein a mean content of the pigment at a portion spaced apart by 10 µm from the surface of the support is at least 33 wt.% and a mean pigment content in the support as a whole is from 10 to 25 wt.%. The present invention can obtain heat-sensitive recording paper for effecting recording by a thermal head or a thermal pen, particularly heat-sensitive recording paper which is free from sticking between a thermal head and a heat-sensitive coloring layer and piling to a thermal head, has high reproducibility of dots even in a high speed recording, has high runability and moreover, can provide clear and high density recording.

## Description

### TECHNICAL FIELD

The present invention relates to heat-sensitive recording paper in which a means such as a thermal head or a thermal pen is used for recording and in particular to heat-sensitive recording paper which does not show sticking between a thermal head and a heat-sensitive color developing layer and piling on the thermal head, which can provide high dot-reproduction and good runnability even during high speed recording and which can also provide clear recorded matters of high density.

### BACKGROUND ART

Heretofore, there has been used coated paper, which has an under coat of a pigment, as a substrate for heat-sensitive recording paper.

The coated paper has good surface smoothness and can provide improved dot reproduction, but suffers from a problem that it requires the use of a large number of manufacturing processes and the production cost thereof is correspondingly increased.

For this reason, there has been a strong need for the development of a technique which makes it possible to simplify the process for preparing such coated paper while maintaining the foregoing advantages of the coated paper. However, there has not been proposed any satisfactory heat-sensitive recording paper unless an under coat is employed.

Accordingly, an object of the present invention is to provide, without using any under coat, heat-sensitive recording paper which exhibits characteristic properties comparable to those of the recording paper having an under coat and which makes it possible to reduce the number of production processes.

### DISCLOSURE OF THE INVENTION

The inventors of this invention have conducted intensive studies to achieve the foregoing object, have found out that the foregoing object can effectively be attained by comprising an invention so as to have the following construction and thus have completed the present invention.

The heat-sensitive recording paper of the present invention comprises a substrate provided thereon with a heat-sensitive color developing layer which comprises a colorless or slightly colored leuco compound and a developer which causes the color development of the leuco compound upon being heated, wherein the content of a pigment in the surface region of the substrate having a thickness of 10 µm is not less than 33% by weight on the average and the substrate has, on the average, an overall content of the pigment ranging from 10 to 25% by weight.

Incidentally, in the conventional recording paper, a pigment is generally uniformly distributed throughout the substrate in order to achieve uniform printing with an ink on both sides of the paper. On the other hand, in the present invention, the distribution of a pigment in the substrate is compulsorily made non-uniform unlike the conventional technique and the recording paper can thus be improved so as not to cause any sticking and piling. The present invention can be completed on the basis of such a finding

### DETAILED EXPLANATION OF THE INVENTION

The present invention will be explained in more detail below.

Preferred examples of the pigments used in the present invention include inorganic pigments such as talc, clay, kaolin, calcined kaolin, synthetic silica and barium sulfate; and organic pigments such as polystyrene resin, polyethylene resin and acrylic resin. The particle size of these pigments is desirably not more than 10 µm.

Regarding the distribution of a pigment in the substrate, the content thereof in the surface region of the substrate having a thickness of 10 µm is not less than 33% by weight on the average and the substrate has, on the average, an overall content of the pigment ranging from 10 to 25% by weight. If the content thereof in the surface region of the substrate having a thickness of 10 µm is not less than 33% by weight on the average, there can be obtained a substrate which exhibits effects comparable to those achieved by the substrate provided thereon with an under coat, that is, it does not cause any sticking and piling and it is substantially improved in dot reproduction during high speed recording.

On the other hand, the content of the pigment in the entire substrate must be, on the average, in the range of from 10 to 25% by weight. This is because, if the overall content thereof is less than 10% by weight, not only the absorbing capacity of the resulting substrate is lowered, but also the adhesion of dregs thereto is increased, while if it is more than 25% by weight, the resulting substrate is limp.

Those skilled in the art can, if necessary, control the distribution of pigments in the substrate by appropriately adjusting factors such as the freeness of pulp, the degree of water-absorbing power of a paper machine and the amount of a fixing agent used.

The distribution of a pigment in the surface region of the substrate having a thickness of 10 µm is in general determined as follows.

First, tapes having a known weight (and the same area as that for the substrate) were adhered to both sides of the material for the substrate having a known weight (and a known thickness), were pulled toward the directions opposite to one another (i.e., at an angle of 180 °) to separate the material for the substrate into two portions and the weight of each separated material was determined. Then a tape was adhered to the side of each portion on which a tape was not present, the tapes were likewise pulled toward the opposite directions to further separate the portion into two portions and the weights of these portions were determined. These operations were repeated 5 to 6 times depending on the proportional allotment of the weight of the portions to separate the material into fractions. The fractions were then ashed by heating them at 600 ° C for 6 hours in an electric furnace. In this case, the material was ashed together with the tape adhered thereto and the weight of the material (each fraction) was determined by subtracting the weight of the ash derived from the tape from the total weight of the resulting ash. The weight of the ash derived from each fraction was plotted against the thickness of the material while assuming that the weight of the fraction is in proportion to the thickness in the substrate to give a graph and thus the rate of the pigment present in the surface region having a thickness of 10 µm could be drawn from the resulting graph.

The substrate used in the present invention mainly comprises wood pulp, but may further comprise synthetic fibers or synthetic pulp. As the wood pulp, there may be used either softwood pulp or hardwood pulp. The freeness of the pulp preferably ranges from 200 to 500 mℓ (C.S.F.) and more preferably 300 to 400 mℓ (C.S.F.). The thickness of the substrate in general ranges from 30 to 100µm and preferably 40 to 80 µ m. The term "thickness of the substrate" herein means that determined immediately after calendering following the paper making.

The substrate may comprise a variety of additives such as sizing agents. Examples of such additives are sizing agents such as rosin, paraffin waxes, higher fatty acid salts, alkenyl succinates, fatty acid anhydrides, styrene/maleic anhydride copolymers, alkyl ketene dimers and epoxidated fatty acid amides; softening agents such as reaction products of maleic anhydride copolymers and polyalkylene polyamines and quaternary ammonium salts of higher fatty acids; agents for strengthening paper such as polyacrylamides, starches, polyvinyl alcohols, melamine/formaldehyde condensates and gelatins; fixing agents such as aluminum sulfate and polyamide polyamine epichlorohydrin. In addition to the foregoing additives, the substrate may further comprise, if necessary, other components such as dyes, fluorescent dyes and antistatic agents.

The heat-sensitive color developing layer in general comprises a colorless or slightly colored leuco dye, a developer, a binder and additives optionally incorporated such as a pigment, a sensitivity controlling agent, an ultraviolet absorber and an antioxidant.

Examples of such leuco dyes include a variety of derivatives such as triphenylmethane derivatives, triphenylmethane phthalide derivatives, fluoran derivatives, leuco-auramine derivatives, diphenylmethane derivatives, phenothiazine derivatives, phenoxazine derivatives, spiropyran derivatives, indoline derivatives and indigo derivatives.

Specific examples thereof suitably used in the invention are as follows (the color observed after color development is given in the parenthesis):
Crystal Violet lactone (blue), 3-diethylamino-6-methyl-7-anilinofluoran (black), 3-dibutylamino-6-methyl-7-anilinofluoran (black), 3-N,N-ethylisoamylamino-6-methyl-7-anilinofluoran (black), 3-(N -ethyl-p-toluidino)-6-methyl-7-anilinofluoran (black), 3-diethylamino-6-methyl-7-(o-, p-dimethylanilino)fluoran (black), 3-pyrrolidino-6-methyl-7-anilinofluoran (black), 3-piperidino-6-methyl-7-anilinofluoran (black), 3(N-cyclohexyl-N-methylamino)-6-methyl-7-anilinofluoran black), 3-diethylamino-7-(o-chloroanilino)fluoran (black), 3-diethylamino-7-(m-trifluoromethylanilino)fluyoran (black), 3-diethylamino-6-methyl-chlorofluoran (red), 3-diethylamino-6-methyl-fluoran (red), 3-cyclohexylamino-6-chlorofluoran (orange) and 3-(N-isoamyl-N-ethylamino)-6-methyl-7-anilinofluoran (black).

The developers used in the present invention are preferably organic acids or esters thereof which are in the solid state at ordinary temperature, melt upon heating and develop a color through the contact with the leuco compound. Preferred examples thereof include various kinds of phenolic compounds, fatty acids, aromatic carboxylic acids or esters thereof.

In the present invention, the amount of the foregoing organic acids in general ranges from 1 to 40% by weight on the basis of the total solid content of the heat-sensitive recording layer. If the amount thereof is limited to the range defined above, the various objects of the present invention can effectively be achieved.

Specific examples of the developers used herein are as follows:
Gallic acid, salicylic acid, 1-hydroxy-2-naphthoic acid, o-hydroxybenzoic acid, m-hydroxybenzoic acid, 2-hydroxy-p-toluic acid, 3, 5-xylenol, thymol, p-tert-butylphenol, 4-hydroxyphenoxide methyl-4-hydroxybenzoate, 4-hydroxyacetophenone, α-naphthol, β-naphthol, catechol, resorcin, 4-tert-octylcatechol, 4,4'-sec-butylidenephenol, 2, 2'-dihydroxydiphenyl, 2,2'-methylenebis(4-methyl-6-tert-butylphenol), 2, 2'-bis(4-hydroxyphenyl)propane (so-called bisphenol A), 4,4'-isopropylidene-bis(2-tert-butylphenol), pyrogallol, fluoroglycine, fluoroglycine carboxylic acid, p-methylphenol, p-tert-butylphenol, p-phenylphenol, 4,4'-cyclohexylidenediphenol, 4,4'-(1-methyl-n-hexylidene)diphenol, 4,4'-(isopropylidene)dicatechol, 4,4'-benzylidenediphenol, 4,4'-isopropylidenebis(2-chlorophenol), 3-phenylsalicylic acid, 3,5-di-tert-butylsalicylic acid, 1-oxy-2-naphthoic acid, gallates, salicylates and 4-hydroxyphthalates.

In the present invention, any known binders may be used. It is preferred to use those soluble in water.

The binders serve to bind the leuco dye which is dispersed in the heat-sensitive recording layer in the form of fine particles while keeping the particles apart from one another.

Preferred examples of the binders used herein are polyvinyl alcohol, methyl cellulose, carboxymethyl cellulose, hydroxyethyl cellulose, polyacrylic acid, casein, gelatin, starches and derivatives thereof.

The amount of these binders ranges from 1 to 35% by weight and preferably 10 to 30% by weight on the basis of the total solid content of the heat-sensitive color developing layer. The various objects of the present invention can effectively be achieved by adjusting the amount of the binder to the range defined above.

Examples of additives which may optionally be incorporated into the heat-sensitive recording layer of the present invention are inorganic and organic pigments such as clay, silica, calcium carbonate, aluminum hydroxide, talc, titanium oxide and zinc oxide; waxes; antioxidants and ultraviolet absorbers for ensuring storage stability; a variety of metal salts of fatty acids for preventing sticking; agents for improving water resistance; phenol resins; and surfactants.

The coating solution for forming the heat-sensitive recording layer is prepared by pulverizing a leuco dye or a developer in an aqueous medium containing a binder such as polyvinyl alcohol in a proper concentration using a pulverizer such as a ball mill or a sand grinder to disperse the same in the aqueous medium and then mixing the resulting dispersions of the leuco dye and the developer together and stirring the mixture. Each constituent substance must be pulverized as fine as possible from the viewpoint of color developing efficiency and hence the constituent substances are preferably pulverized into particles having a particle size ranging from 0.5 to 3 µm. The heat-sensitive paint thus prepared is applied onto a substrate in the usual manner using a blade coater, an air knife coater, a bar coater or a reverse roll coater and then dried to give the heat-sensitive recording paper according to the present invention.

### EXAMPLES

The present invention will be described in more detail with reference to the following Examples.

### Example 1

To a pulp slurry consisting of 50 parts by weight of LBKP having a C.S.F. freeness of 300mℓ and 50 parts by weight of NBKP having a C.S.F. freeness of 300mℓ, there were added 70 parts by weight of precipitated calcium carbonate (PC; available from Shiraishi Kogyo Kaisha, Ltd.), 6 parts by weight of a cationized starch (available from Nippon Starch Chemical Co., Ltd.), 0.5 part by weight of an anionic polyacrylamide (Polystron 117; available from Arakawa Chemical Industries, Ltd.) and 1 part by weight of a sizing agent for neutral (Hercon W; available from Dick Hercules Co., Ltd.), the resulting slurry was formed into paper and then subjected to calendering to give paper having a thickness of 66 µ m, a basis weight of 55 g/m² and a surface smoothness of 600 sec. Thus, there was obtained a substrate having a degree of sizing of 18 sec, the pigment content of 10% by weight and the pigment content of the surface region having a thickness of 10 µm of 35% by weight.

Then the following solutions A, B and C were separately prepared and there were mixed 52 parts by weight of the solution A, 90 parts by weight of the solution B and 56 parts by weight of the solution C as well as 20 parts by weight of a 30% dispersion of zinc stearate and 125 parts by weight of a 12% aqueous solution of polyvinyl alcohol to give a coating solution for forming heat-sensitive recording layers.

The solutions A and B were separately dispersed for 16 hours using a paint conditioner.

The solution C was dispersed for 10 minutes with a homomixer. The resulting coating solution was applied onto the foregoing paper substrate so that the amount thereof coated was equal to 6 g/m², dried and then subjected to calendering so that the Bekk surface smoothness was equal to about 600 sec to give heat-sensitive recording paper.

### Examples 2 to 6 and Comparative Examples 1 to 4

The same procedures used in Example 1 were repeated except that the overall distribution of a pigment and that in the surface area having a thickness of 10 µm were changed to those listed in the following Table-1 to give each corresponding heat-sensitive recording paper.

### Example 7

To a pulp slurry consisting of 50 parts by weight of LBKP having a C.S.F. freeness of 300mℓ and 50 parts by weight of NBKP having a C.S.F. freeness of 300mℓ, there were added 50 parts by weight of kaolin of secondary grade, 0.5 part by weight of an anionic polyacrylamide (Polystron 117; available from Arakawa Chemical Industries, Ltd.) 0.6 parts by weight of a rosin type sizing agent (available from Harima Chemicals, Inc.) and 2.5 parts by weight of aluminum sulfate, the resulting slurry was formed into paper and then subjected to calendering to give paper having a thickness of 60 µm, a basis weight of 55 g/m² and a surface smoothness of 600 sec. Thus, there was obtained a substrate having a degree of sizing of 15 sec, the pigment content of 20% by weight and the pigment content of the surface region having a thickness of 10 µm of 40% by weight. Then the same procedures used in Example 1 were repeated to give heat-sensitive recording paper.

### Comparative Example 5

A 25% solution containing 40 parts by weight of PVA (Poval 105; available from Kuraray Co., Ltd.) and 100 parts by weight of silica (P 527; available from Mizusawa Industrial Chemicals, Ltd.) was applied onto the paper prepared in the same manner used in Example 1 except that any calcium carbonate was not used in an amount of 6 g/m² and then the same coating solution for heat-sensitive layers used in Example 1 was applied thereto to give heat-sensitive recording paper.

With the heat-sensitive recording paper obtained in the foregoing Examples and Comparative Examples, printing operation was performed using a commercially available G facsimile apparatus FACOM FAX 621C (available from Fujitsu Limited) under the following conditions: electric power for recording of 0.90 W/dot; time of turning on electricity of 0.45 msec; and a period of about 5 msec and the density of the resulting images and that of the background after printing were determined using a Macbeth densitometer. Moreover, the dot reproduction was also evaluated visually.

As regard to the runnability, solid printing was performed using Thermal Printer VP-35 available from Seiko Co., Ltd. and the sticking was estimated in terms of the sticking noises observed during the solid printing and further an image of A-4 having a black rate of 50% was recorded 1000 times using FACOM FAX 2000 available from Fujitsu Limited to determine whether defects such as jamming are observed or not.

As seen from the results listed in the following Table-1, there can be obtained heat-sensitive recording paper which makes it possible to prevent the sticking and piling and which can provide excellent dot reproduction during high speed recording, if the average content of pigment in the surface region of a substrate having a thickness of 10 µ m is controlled to not less than 33% by weight and the overall content thereof in the substrate is adjusted to the range of from 10 to 25% by weight.

## Claims

1. Heat-sensitive recording paper comprising a substrate provided thereon with a heat-sensitive color developing layer which comprises a colorless or slightly colored leuco compound and a developer which causes color development of the leuco compound upon being heated, wherein the content of a pigment in the surface region of the substrate having a thickness of 10 µm is not less than 33% by weight on the average and the substrate has, on the average, an overall content of the pigment ranging from 10 to 25% by weight.

2. Heat-sensitive recording paper of claim 1 wherein the thickness of the substrate ranges from 30 to 100µm.

3. Heat-sensitive recording paper of claim 1 wherein the thickness of the substrate ranges from 40 to 80 µm.

4. Heat-sensitive recording paper of claim 1 wherein the pigment is a member selected from the group consisting of talc, clay, kaolin, calcined kaolin, synthetic silica, barium sulfate, polystyrene resin, polyethylene resin and acrylic resin.

5. Heat-sensitive recording paper of claim 4 wherein the particle size of the pigment is not more than 10µm.
